

## UNITED STATES PATENT OFFICE

2,013,689

## TREATMENT OF TEXTILE MATERIALS

Ernest William Kirk and George Holland Ellis,  
Spondon, near Derby, England, assignors to  
Celanese Corporation of America, a corporation  
of Delaware.

No Drawing. Application April 14, 1933, Serial  
No. 666,173. In Great Britain May 12, 1932

7 Claims.

(Cl. 8—5)

This invention relates to the production of colorations on textile materials and especially upon materials consisting of or containing cellulose acetate or other cellulose esters or ethers.

5 In the coloration of textile materials it is frequently found necessary, in order to obtain a particular shade or a particular shade of special fastness or other property, to employ mixtures of coloring matters. In general however it is necessary, unless the coloring matters are of closely related dyeing properties, to apply the component dyestuffs in separate operations. Thus in order to produce compound shades from vat dyestuffs on the one hand and azoic colors (i. e. insoluble azo dyes formed on the material) on the other, it has generally been regarded as necessary to apply the colorations in separate operations owing to the great difference between the necessary procedures in the two cases.

20 We have now found that valuable mixed shades may be obtained by applying to or incorporating in textile materials a leuco compound of a vat dyestuff, a diazotizable amine and an azo coupling component, and thereafter subjecting the material to treatment to effect diazotization and coupling, and also the oxidation of the leuco compound to the parent vat dyestuff.

25 Thus, for example, a cellulose acetate material may be dyed in a green shade by impregnating with a chloraniline and diacet-o-acetyl-ortho-tolidide and the leuco compound of a blue indigoid dyestuff and thereafter treating with nitrous acid in order to diazotize the amine and so effect coupling, and simultaneously to oxidize the leuco compound of the vat dyestuff. In this way the desired mixed shades of vat and azoic colors may be obtained with little or no more complication of procedure than is normally necessary in the production of azoic colorations on textile materials.

35 Moreover, the mixed shades obtainable exhibit a high degree of fastness for the dyeings obtainable by vat or azoic methods in general exhibit exceedingly good fastness properties.

40 The three components, diazotizable amine, coupling component and leuco vat dyestuff, are conveniently applied to the material simultaneously from a single bath, padding liquid or the like. If desired however they may be applied separately to the materials, though in general less conveniently.

45 The diazotization of the amine and subsequent coupling and the oxidation of the leuco compound to the vat dyestuff may be effected in any convenient way. Thus, for instance the impregnated material may be subjected to a mild oxida-

tion, for example, by means of air, in order to oxidize the leuco compound, and thereafter to the action of nitrous acid, followed if necessary by an alkaline treatment, in order to effect diazotization and coupling. Most conveniently however the diazotization and oxidation of the leuco compound are effected simply by treatment in a nitrous acid bath, the nitrite serving the dual purpose of diazotizing agent and oxidizing agent. Following the nitrous acid treatment the materials may be subjected to soaping, preferably in the presence of sodium carbonate, or to other weak alkaline treatment to ensure completion of the coupling. Further, if desired, the material may be subjected to a mild oxidizing treatment to ensure the complete oxidation of the leuco compound of the vat dyestuff.

50 The diazo component, coupling component and leuco vat dyestuff, may be applied to the materials either in the free state or in the form of salts, according to the character of the material undergoing treatment and the precise method of application employed. Thus, in the case of cellulosic materials the coupling component and the leuco compound are advantageously applied in the form of alkali salts, in which form they exhibit very good affinity for the material. In the case of animal fibres, for example wool or silk, and cellulose acetate or other cellulose ester or ether artificial silks, the components are, with particular advantage, applied in the free state to the materials. In this state the components exhibit very good affinity for these materials, and in consequence dyeings are obtained possessing very good fastness to rubbing, in addition to other desirable fastness properties.

55 If desired leuco compounds of the vat dyestuffs may be applied to or incorporated in the materials in the form of their sulphuric, phosphoric or other esters, for example the products sold under the name Indigosol or the registered trade-mark Soledon. These sulphuric or other esters of the leuco compounds are readily saponified and oxidized to the vat dyestuff by the nitrous acid baths suitable for effecting the diazotization of the amines. When therefore these esters are employed the treatment may be similar to that adopted when the leuco vat dyestuffs are employed in the free state or in the form of alkali metal salts.

60 Diazotizable amines of any desired character may be employed, for example primary amines of the benzene, naphthalene, carbazole, anthra-quinone and other series. Examples of suitable

5

10

15

20

25

30

35

40

45

50

55

amines are given for instance in U. S. Patent No. 1,844,350, British Patents 396,412 and 404,327.

Likewise coupling components of widely varying character may be employed, for example any 5 of those mentioned in U. S. application S. No. 666,172, for example arylamides of 2:3-oxynaphthoic acids. Particularly useful results may be obtained by using diacylacetyl derivatives of aromatic diamines in conjunction with blue to 10 green vat dyestuffs whereby valuable bright green shades may be produced. Thus such a green may be produced from Algol brilliant green BK (Schultze 7th Edition, volume 2, page 6), diaceto-acetyl-orthotolidide and orthochloraniline. Again, purple shades may be obtained by 15 using 5:7:5':7'-tetrabromindigo, 2:3-oxynaphthoic acid-*m*-nitranilide and 5-nitro-2-aminoanisole.

The vat dyestuffs employed may be of any desired series, for example of the anthraquinone or indigoid series. Further, sulphur dyestuffs may be applied in accordance with the new process, and in fact any of the dyestuffs or classes of dyestuffs referred to in U. S. Patent No. 1,960,172 20 as suitable for application to cellulose ester and ether materials in the form of their free leuco compounds. In the case of cellulose ester or ether materials, particularly useful results may be secured by means of dyestuffs of the indigoid 25 series, or by means of anthraquinone dyestuffs containing only a single anthraquinone nucleus.

Dispersions of the diazo or coupling components may be obtained by any desired method, for example, by fine milling or grinding with or without the aid of dispersors and/or protective colloids, by precipitation in the presence of protective colloids, or by a simple treatment with dispersors, as described for instance in any of U. S. Patents Nos. 1,618,413, 1,618,414, 1,694,413, 35 40 1,690,481, 1,803,008, 1,840,572, 1,716,721 and 1,928,647 and British Patent No. 323,788. Dispersion of coupling components, especially those of phenolic character or containing the  $-\text{CO}.\text{SH}_2-$  group may frequently be facilitated by the presence of small quantities of alkali, for example, a 45 quantity of caustic soda sufficient to yield a solution of about pH7.2 or even slightly more alkaline.

Vat dyestuffs may be vatted with caustic alkali and a reducing agent and applied to the 50 materials together with or separately from the diazo and coupling components. In the case of animal fibres, cellulose esters or other materials liable to damage by alkali, the excess alkali of the vat may be neutralized, for example by means 55 of organic acids or there may be used vats of relatively low alkalinity prepared with the aid of ammonia, organic amines or other weak alkalies. Any such organic acids or organic bases should of course be such as do not interfere with 60 the production of the desired shades, e. g., by coupling with the diazo compound. Where the leuco compounds are to be applied to the materials in the free state they are advantageously converted into fine suspensions or dispersions, 65 for example in any of the ways described in U. S. Patent No. 1,900,172.

The various components, whether in free or combined form, may be applied to the materials in any desired manner. Thus, for instance, 70 they may be applied by dyeing, padding or other mode of uniform application, or by printing, stencilling or other mode of local application. For padding, printing and the like the preparations containing the components may contain any 75 desired thickening or other agents to fit them

for the particular method of application employed. Steaming may be utilized if desired, in order to fix components or coloring matters on the materials, more particularly when such components or coloring matters have been applied by printing, padding or other form of mechanical impregnation. If desired, one component may be applied uniformly to the material and another component locally to the material, whereby valuable two-color effects may be obtained. Thus, 10 for example, material may be uniformly impregnated with a mixture of diazotizable amine and coupling component, over-printed with a leuco compound of a vat dyestuff or an ester thereof and thereafter diazotized and developed. 15 In this way a pattern colored by both dyestuffs is obtained upon a ground colored only by the azoic colorations.

As indicated previously the invention is of especial interest in the coloration of cellulose 20 ester or ether materials. Such materials may for instance consist of the previously mentioned cellulose acetate or of other cellulose esters or mixed esters, for example cellulose formate, propionate, butyrate, a nitroacetate, or acetate-butyrate, or 25 cellulose esters obtained by esterifying cellulose while retaining its fibrous form. Again, cellulose ethers, or ether-esters for instance ethyl or benzyl cellulose may be colored. Other natural or artificial materials, for example animal fibres, 30 cotton or the regenerated cellulose type of artificial silk may likewise be colored by the new process. Again, the method may be applied to mixed materials comprising two or more of the above-mentioned fibres. The components of such mixed 35 materials may be colored in solid or contrasting shades according to their respective affinities for the components under the conditions of application. For example, in the case of a material consisting of cellulose acetate and a cellulosic fibre 40 such as cotton or viscose artificial silk, the acetate only may be colored by applying the components in the free state, under which conditions they possess little or no affinity for the cellulosic material.

The invention is illustrated but not limited by the following examples:—

#### Example 1

To dye a brilliant emerald green shade on 10 50 kilograms of cellulose acetate yarn.

300 grams of Algol brilliant green BK paste (Schultze, 7th Edition, volume 2, page 6) are wetted down with methylated spirit and vatted in about 30 litres of soft water at 60° C. by addition 55 of 50 ccs. of monoethanolamine and 100 grams of sodium hydrosulphite powder. In another vessel 100 grams of ortho-chloraniline are dispersed by heating with 200 grams of Turkey red oil and diluting with hot soft water. Both these solutions 60 are then added to the dyebath, followed by a solution of 200 grams of diaceto-acetyl-ortho-tolidine in sufficient hot soft water containing 40 grams of caustic soda. A solution of 100 grams of glucose is then added and the bath adjusted to 65 300 litres. The yarn is entered into the dyebath at 30-40° C. and worked for half-an-hour, during which time the temperature of the bath is raised to 75° C. and the dyeing continued at this temperature for a further hour. The yarn is 70 lifted, thoroughly rinsed off, and entered in a diazotization bath containing 8 grams per litre of glacial acetic acid and 4 grams per litre of sodium nitrite, the temperature not exceeding 15° C. After working in this bath for half-an-hour the 75

yarn is again lifted and thoroughly rinsed, and then entered into a cold bath containing  $\frac{1}{4}$  gram per litre soda ash and 1 gram per litre good textile soap, worked cold for a quarter of an hour, 5 the temperature raised slowly to 75° C. and worked at this point for a further half hour. The yarn is then lifted, rinsed and dried, or otherwise treated as requisite.

10 *Example 2*

To obtain a green printed design on a white ground of cellulose acetate fabric.

The following paste is first prepared:—

15 1.6 parts 2:5-dichloraniline  
3.8 " Diacetooctylorthotolidine.  
6.0 " Indigosol blue AZG.  
10.0 " Ethyl lactate.  
10.0 " Diethylene glycol.  
20 Gum arabic thickening to  
100.0 parts

The fabric is printed with the above paste, dried at a moderate temperature, steamed at 5 lbs. per square inch pressure in the "Cottage" 25 steamer for 20 minutes and then treated for half-an-hour at 50° C. in a bath containing 8 grams per litre of sodium nitrite and 16 grams per litre glacial acetic acid, rinsed, soaped at 75° C. for 20 minutes, again rinsed and dried or otherwise finished as requisite.

30 *Example 3*

To dye a fast green shade on 10 kilograms of silk yarn.

35 100 grams of 5:7:5':7' tetrabromindigo are vatted by warming to 60° C. with 200 grams of monoethanolamine, 200 grams Turkey red oil and 100 grams of sodium hydrosulphite in 5 litres of soft water. 100 grams of 2:5-dichloraniline are dispersed by warming with 300 ccs. of Turkey red oil and diluting with 1 litre of boiling soft water, and 200 grams of di-aceto-acetyl-orthotolidine are dissolved with 50 grams of caustic soda and 5 litres of hot soft water. 40 These dispersions are then added to the dyebath which already contains 100 grams of glucose and which is adjusted to a volume of 300 litres, and the previously degummed silk yarn entered. The temperature is then slowly raised to 75° C. and kept at this for an hour and a half, the silk meanwhile being well turned. The yarn is then lifted and rinsed, and entered directly into the diazotizing bath which contains 6 grams of sodium nitrite and 12 ccs. of glacial acetic acid per litre. After 45 diazotization for 15 minutes, the yarn is lifted, rinsed, and soaped to shade as in Example 1 above, and again lifted and rinsed or otherwise treated as necessary.

50 What we claim and desire to secure by Letters Patent is:—

55 1. Process for the production of mixed shades on textile materials, which comprises applying to the materials a diazotizable amine, an azo coupling component and a compound selected from the group consisting of the free leuco compounds of vat dyestuffs and the salts of the free leuco compounds of vat dyestuffs, and thereafter simultaneously effecting diazotization and coupling and conversion of the leuco derivative to the parent vat dyestuff with nitrous acid.

60 2. Process for the production of mixed shades

on textile materials containing organic derivatives of cellulose, which comprises applying thereto a diazotizable amine, an arylamide of 2,3-oxy-naphthoic acid, and a compound selected from the group consisting of the free leuco compounds 5 of vat dyestuffs and the salts of the free leuco compounds of vat dyestuffs, and thereafter simultaneously effecting diazotization and coupling and conversion of the leuco derivative to the parent vat dyestuff with nitrous acid. 10

3. Process for the production of mixed shades on textile materials containing organic derivatives of cellulose, which comprises applying to the materials a diazotizable amine, an azo coupling component, and a compound selected from the group 15 consisting of the free leuco compounds of vat dyestuffs and the salts of the free leuco compounds of vat dyestuffs, and thereafter simultaneously effecting diazotization and coupling and conversion of the leuco derivative to the parent vat dye- 20 stuff with nitrous acid.

4. Process for the production of mixed shades on textile materials containing cellulose acetate, which comprises applying thereto a diazotizable amine, a diacyl-acetyl derivative of an aromatic 25 diamine, and a compound selected from the group consisting of the free leuco compounds of vat dyestuffs and the salts of the free leuco compounds of vat dyestuffs, and thereafter simultaneously effecting diazotization and coupling and 30 conversion of the leuco derivative to the parent vat dyestuff with nitrous acid.

5. Process for the production of mixed shades on textile materials containing organic derivatives of cellulose, which comprises applying to the 35 materials a diazotizable amine, an azo coupling component and a compound selected from the group consisting of the free leuco compounds of anthraquinone vat dyestuffs containing a single 40 anthraquinone nucleus, and the salts of said free leuco compounds, and thereafter simultaneously effecting diazotization and coupling and conversion of the leuco derivative to the parent vat dyestuff with nitrous acid.

6. Process for the production of mixed shades 45 on textile materials containing cellulose acetate, which comprises applying to the materials a diazotizable amine, an azo coupling component and a compound selected from the group consisting of the free leuco compounds of anthraquinone vat 50 dyestuffs containing a single anthraquinone nucleus, and the salts of said free leuco compounds, and thereafter simultaneously effecting diazotization and coupling and conversion of the leuco derivative to the parent vat dyestuff with nitrous acid.

7. Process for the production of mixed shades on textile materials containing cellulose acetate, which comprises applying to the materials a diazotizable amine, a diacyl-acetyl derivative of an 60 aromatic diamine, and a compound selected from the group consisting of the free leuco compounds of anthraquinone vat dyestuffs containing a single 65 anthraquinone nucleus and the salts of said free leuco compounds, and thereafter effecting diazotization and coupling simultaneously with conversion of the leuco derivative to the parent vat dyestuff with nitrous acid.

CERTIFICATE OF CORRECTION.

Patent No. 2,013,689.

September 10, 1935.

ERNEST WILLIAM KIRK, ET AL.

It is hereby certified that error appears in the printed specification of the above numbered patent requiring correction as follows: Page 2, first column, lines 5 and 6, for "U.S. Application S. No. 666,172" read British Patent No. 404,327; and that the said Letters Patent should be read with this correction therein that the same may conform to the record of the case in the Patent Office.

Signed and sealed this 8th day of October, A. D. 1935.

(Seal)

Leslie Frazer  
Acting Commissioner of Patents.